

N. E. CLARK,  
CONCRETE REINFORCEMENT,  
APPLICATION FILED JUNE 22, 1908.

1,138,932.

Patented May 11, 1915.



WITNESSES:

C. H. Berthoff  
Frank R. Dillinger.

INVENTOR  
Norris Elmore Clark.

BY  
R. D. Lynn  
ATTORNEY

# UNITED STATES PATENT OFFICE.

NORRIS ELMORE CLARK, OF PLAINVILLE, CONNECTICUT.

## CONCRETE REINFORCEMENT.

1,138,932.

Specification of Letters Patent. Patented May 11, 1915.

Application filed June 22, 1908. Serial No. 438,848.

*To all whom it may concern:*

Be it known that I, NORRIS ELMORE CLARK, a citizen of the United States, residing at Plainville, in the county of Hartford and State of Connecticut, have invented certain new and useful Improvements in Concrete Reinforcement, of which the following is a specification.

My invention relates particularly to 10 metallic fabrics for reinforcing concrete and cement structures.

The main object is to provide an expanded metal fabric having parallel rod or bar members so formed as to be strong and 15 have a good holding capacity in the concrete.

Another object is to provide as much 20 strength and holding power as possible with a given quantity of metal.

25 The rod members in the form shown are deformed by twisting adjacent sections in reverse directions. The rod or bar members are deformed for instance by twisting so as to increase the bonding effect in the concrete 25 and prevent the formation of lines of cleavage.

30 By working the rod or bar members while cold the elastic limit is increased so that the fabric performs its reinforcing function with greater efficiency.

The drawing shows a plan view of an 35 expanded metal fabric embodying one form of my invention.

The fabric as shown is formed by slitting a sheet of metal, expanding it so as to separate the bars 1, 1, 1, and leaving them connected integrally by the strands such as 12, 13 and 14, 15. Each bar is then twisted as for instance by applying stationary jaws 40 to the points 16 and 17, and a rotating jaw to the point 18. This produces oppositely twisted helices on the opposite sides of the point 18 as shown. The section from 17 to 19 is then twisted in similar manner and 45 so also the sections of the other bars. Thus an expanded metal fabric may be produced, the longitudinal tension bars of which have

a higher elastic limit than is possible by any other method. By this construction the longitudinal parallel bar or rod members are deformed so as to give a better bonding effect and prevent slipping and the formation of lines of cleavage in the concrete. By twisting the bars or rod members while cold their elastic limit is increased above that of the strands or tie members 50 12 and 13 so that while the bars are stiffer, the strands or ties of the reticulated sections are still more or less flexible so as to give greater capacity for expansion 55 and contraction in the reticulated portions.

What I claim is:

1. An expanded metal reinforcing fabric comprising parallel tension members and bent tie members forming meshwork integrally connecting adjacent tension members, the said tension members having an elastic limit greater than that of the tie members.

2. An expanded metal reinforcing fabric 70 comprising twisted bar members and tie members integrally connecting adjacent twisted bar members.

3. An expanded metal reinforcing fabric comprising parallel bar members with deformation at the sides for bonding engagement in concrete and bent tie members integrally connecting adjacent bar members and forming a mesh-work, the bar members having higher elastic limit than the tie members.

4. A reticulated reinforcing fabric for concrete comprising longitudinal parallel bar members having lateral deformation for affording bonding engagement in the concrete and reticulated sections integrally connecting the adjacent edges of adjacent bar members, the bar members having a materially higher elastic limit than the metal of the reticulated sections.

NORRIS ELMORE CLARK.

Witnesses:

E. BRADFORD,  
ROBT. G. ALLYN.